

May 29, 1973

D. W. GOSSELINK ET AL

3,736,134

HUMIDITY RESISTANT PHOTOCONDUCTIVE COMPOSITIONS

Filed Oct. 14, 1970



INVENTORS  
DONALD W. GOSSELINK  
EINAR D. HORNE  
BY *Kinney, Alexander,  
Sell, Steldt & DeLaHunt*  
ATTORNEYS

## 1

3,736,134

## HUMIDITY RESISTANT PHOTOCONDUCTIVE COMPOSITIONS

Donald W. Gosselink, North St. Paul, Minn., and Einar D. Horne, Hudson, Wis., assignors to Minnesota Mining and Manufacturing Company, St. Paul, Minn.  
Filed Oct. 14, 1970, Ser. No. 80,567  
Int. Cl. G03g 5/08

U.S. CL. 96—1.8

17 Claims

## ABSTRACT OF THE DISCLOSURE

Improvement in the humidity resistance of photoconductive titanium dioxide containing electrographic elements is achieved by combining therewith a carboxylic acid or metal salt thereof such as abietic acid or zinc abietate with an inorganic metal oxide such as zinc oxide.

This invention relates to photoconductive compositions and more particularly, to photoconductive compositions having improved humidity resistance.

Photoconductive compositions are utilized in numerous electrographic processes both as intermediate and final receptor surfaces for the developer (ink) delineating the subject matter being reproduced. As an integral part of these processes, the photoconductive surface must exhibit particular electrical properties depending upon the characteristics of the electrographic process. Humidity can and often does affect these electrical properties to the extent that a photoconductive surface suitable in a particular electrographic process at one humidity may be unsuitable at a different humidity. In general, it is at high relative humidities that the quality of reproduction deteriorates, often to the point that little or no image definition is obtained.

It is entirely too expensive to control humidity by external means, particularly for electrographic processes employed for general copying. This invention relates to a composition and technique for improving humidity resistance at the source by providing an improved humidity resistant photoconductive composition.

Exemplary electrographic processes are the electrolytic electrophotographic process described in U.S. Pat. No. 3,010,883, the electrostatic electrophotographic processes such as is illustrated by U.S. Pat. No. 3,152,894, and the dynamic electrographic (electropowder) process described in U.S. application Ser. No. 668,183 and French Pat. No. 1,456,993. Although the photoconductive composition of this invention has general applicability to electrographic processes operating on the above principles, it is particularly adapted as an intermediate for the production of multiple copies in the electropowder process.

In this latter process, a photoconductive sheet is used as a field electrode and is exposed to a light image to create a differentially electronically conductive pattern on the field electrode. While the differentially conductive pattern is present in the photoconductive sheet or field electrode, the surface of the field electrode is uniformly contacted with a conductive applicator containing electrically conductive developer or transfer medium while an electrical field is created by applying a direct current electrical potential between the field electrode and the applicator containing the conductive developer. An electrically conductive path is created between the surface of the field electrode and the applicator. Separation of the developer applicator from the field electrode surface at the end of the development stage is made while the electrical field is maintained. The developer selectively deposits on the field electrode surface in an image-wise manner corresponding to the original light image, thus providing a visible reproduction. No electrostatic pre-

## 2

charging of the field electrode surface is either indicated or desirable. If desired, the developer material may be retained on the field electrode surface or may be transferred to a separate receptor sheet and fixed thereon by chemical or physical means to provide the desired print.

The problem of humidity as its affects electrostatic copying is discussed in U.S. Pat. 3,248,217, wherein a humidity resistant photoconductive sheet is disclosed, the photoconductive coating consisting essentially of a photoconductor, generally zinc oxide, an emulsifiable polyethylene binder, a water-insoluble fatty acid, and a water-insoluble dispersant formed from a water-soluble lower alkyl silicone resin. The water-insoluble fatty acids are said to contribute to the water resistance of the final coating. Upon drying and curing of the coating the silicone resins form a water-insensitive coating around the photoconductive zinc oxide particles. It is recognized that silicones in general afford a measure of humidity protection.

In the present invention, certain additives are employed to extend humidity protection to photoconductive titanium oxide. Titanium dioxide has been found to undergo a gradual decrease in image density with increasing humidity as illustrated by the following data:

|                                   | Image density<br>(maximum) |
|-----------------------------------|----------------------------|
| Temp. ° F./Rel. humidity: 72°/40% | 1.09 O.D.U.                |
| 80°/80%                           | 0.76 O.D.U.                |
| 80°/61%                           | 0.                         |

With the use of an inorganic oxide other than titanium dioxide in combination with a carboxylic acid, or salt thereof, the humidity resistance of photoconductive titanium dioxide is improved as will be shown hereinafter.

The photoconductive titanium dioxide, inorganic oxide other than titanium dioxide, and carboxylic acid or salt thereof may be combined with a binder in the form of a coating on a substrate suitable for use in an electrographic process. The characteristics of the substrate will depend on the electrographic process in which the photoconductive composition is to be employed. Belts, sheets, rollers, and drums are typical forms of substrates for photoconductive compositions. In the case of the dynamic electrographic process described in commonly assigned U.S. application Ser. No. 668,183, the photoconductive composition takes the form of a surface coating on a dielectric film to provide an electrographic sheet or field electrode. The electrographic sheet preferably includes an electronically conductive layer bonded to the underside of the dielectric layer, i.e., the face opposing that on which the photoconductive composition is coated.

The accompanying drawing illustrates this preferred electrographic sheet. Referring to the figure, there is shown an electrographic sheet 1 having a photoconductive image layer 3, a dielectric layer 5, and conductive layer 7 bonded to the dielectric layer 5.

The image layer formed from the photoconductive composition of this invention should upon light exposure provide a differentially conductive pattern wherein the conductive regions are at least twice as conductive as the nonconductive regions, preferably at least 10 times as conductive. The relatively conductive regions of the image layer (containing the conductive pattern) should be as conductive as possible and at least have a maximum resistivity at the surface of  $10^{15}$  ohm-cm., preferably  $10^{14}$  ohm-cm. The relatively nonconductive regions should generally have a minimum resistivity at the surface of  $10^7$  ohm-cm., although for special conditions, a resistivity of  $10^4$  or  $10^5$  ohm-cm. would be suitable. These resistivity values are measured under an electric field and for an applied time corresponding to that to be used in the electropowder process, and it is to be remembered that the

conductive regions are at least twice as conductive as the nonconductive regions within the above over-all ranges, and the conductive regions are at least about 10 times as conductive as the dielectric layer. For best results, the limits of transverse resistivity at the surface of both the nonconductive regions and the conductive regions of the electrode are between about  $10^7$  and  $10^{14}$  ohm-cm.

For the preferred embodiment herein where the photoconductive sheet is to be employed in the electropowder process, the base for the photoconductive surface coating comprises a dielectric layer alone or in combination with a conductive layer bonded to the undersurface of the dielectric layer. The conductivity of the dielectric layer should be about  $10^{-11}$  (ohm-cm.) $^{-1}$  or lower, and preferably  $10^{-12}$  or lower, a conductivity fulfilled by most good dielectric or insulating materials. It is preferred that the dielectric layer exhibit such conductivity independent of the ambient conditions, i.e., temperature and relative humidity. In any case, the conductivity of the dielectric layer should be at most about .1 the conductivity of the conductive layer when present.

A variety of materials satisfy the requirements for the dielectric layer of this invention including paper, polyesters such as those available commercially under the trade names Mylar and Scotchpar, polypropylene, polycarbonate, cellulose acetate, and polystyrene. Polyesters are preferred.

The conductive layer may be supporting or non-supporting, for example, a thin vapor coated metal layer or a thicker conductive paper support. Generally, the conductive layer is bonded to the dielectric layer which bears the photoconductive surface layer. For some electrographic processes, the photoconductive composition may be applied directly to a conductive substrate. For the electropowder process, the conductivity of this layer should be such that no more than a small voltage drop occurs across it when the developing current passes through it. Small in this sense is relative to the voltage drop in other parts of the circuit through which current passes. Preferably, the voltage drop across the conductive layer should be no more than about  $\frac{1}{10}$  of the development voltage. Generally, the resistivity of the conductive layer should be less than about  $10^{10}$  ohm-cm., depending upon processing conditions and thickness of the layer. Exemplary conductive materials include conductive paper, paper-metal foil laminates and foils, coatings or other forms of metals such as copper, iron, silver, and aluminum. The conductive layer may be in the form of a plurality of plies of conductive material or a single layer made from a single material or a mixture of materials.

The titanium dioxide employed in the present invention is photoconductive. Preferably, the titanium dioxide is of the type described in commonly assigned U.S. application Ser. No. 867,738 which will enable the production of multiple copies per exposure of the electrographic sheet in the dynamic electrographic process. This titanium dioxide is characterized as having a characteristic relaxation time of less than 9 minutes, and preferably less than 6 minutes. The determination of characteristic relaxation time is fully described in said application Ser. No. 867,738. Employing titanium dioxide exhibiting such a characteristic relaxation time, in combination with the organic acids or salts thereof, has enabled the production of several copies of the original from a single exposure of the electrographic sheet.

Included in the photoconductive composition is a carboxylic acid or salt thereof. In general, carboxylic acids which will convert to the metal salt by reaction with the corresponding metal oxide may be employed. Exemplary carboxylic acids are aliphatic, cycloaliphatic, aromatic acids such as acetic, propionic, butanoic, hexanoic, octanoic, lauric, stearic, benzoic, oleic, cerotic, caproic, linoleic, abietic, rosin acids, dehydroabietic acid, 1-naphthoic, 2-naphthoic, o-nitrobenzoic, and m-nitroben-

zoic acid. The carboxylic acids having two or more atoms may be employed, preferably 2 to 30 carbon atoms, and most preferably 6 to 20 carbon atoms. Exemplary salts are ammonium salts and metal salts. Examples of the latter include alkali metal, alkaline earth metal, aluminum, gallium, and zinc salts. Preferred are the zinc salts of the above mentioned carboxylic acids, especially zinc abietate and zinc rosinate.

Also present in the photoconductive composition is a metal oxide other than photoconductive titanium dioxide, suitable metal oxides including barium oxide, calcium oxide, magnesium oxide, lead (II) oxide, lead (IV) oxide, mercuric oxide and zinc oxide.

The photoconductive titanium dioxide, carboxylic acid or salt thereof, and metal oxide as described herein may be disposed in an insulating binder, generally an insulating resin binder, to provide a coating for an electrographic sheet. Exemplary binders include chlorinated polyethylene, polyvinyl acetate, Lexan polycarbonate, polystyrene, styrene copolymers (e.g., styrene-butadiene copolymer, styrene-n-butyl acrylate copolymer, styrene-isoprene copolymer), acrylonitrile copolymers, polymethyl methacrylate, polybutyl methacrylate, polyhexyl methacrylate, polydimethylaminoethyl methacrylate, polymethyl acrylate, polycyanoethyl acrylate copolymers, and polyvinylidenechloride polymers. Preferably, the binders have an acid number below 70, and most preferably below 40, and are free of emulsifying agents. Preferred polymeric binders are polystyrene-butadiene copolymers, chlorinated polyethylene, polyvinyl acetate and Lexan polycarbonate.

In addition to the foregoing components, the photoconductive composition may contain other additives. One preferred additive is a class of materials known as dye sensitizers. Their concentration should preferably be below  $3 \times 10^{-2}$ , most preferably  $3 \times 10^{-3}$ , grads of dye per gram of titanium dioxide.

The carboxylic acid or salt thereof levels of about  $1.85 \times 10^{-6}$ , preferably  $3.7 \times 10^{-6}$ , equivalents per square meter of titanium dioxide surface have proved suitable. The amount of carboxylic acid or salt thereof may also be expressed in terms of an amount sufficient to provide at least one-half and preferably at least one monomolecular surface coverage of the photoconductive titanium dioxide. The inorganic metal oxide should be present to the extent of at least one-half and preferably at least one chemical equivalent of the carboxylic acid or salt thereof. The amount of inorganic metal oxide may also be expressed as at least .15% by weight based upon the combined weight of titanium dioxide and inorganic metal oxide.

The titanium dioxide should be present to the extent sufficient to provide a developable image in the electrographic process. Generally, the titanium dioxide may be present to the extent of about 20 to about 80 volume percent of the combined volume of titanium dioxide and insulating resin binder, preferably 40 to 60 percent, and most preferably 50-55%.

The following examples are provided to illustrate the invention.

#### EXAMPLES 1-14

A smooth dispersion is prepared by ball milling for 16 hours 38 grams titanium dioxide, 12.6 grams chlorinated polyethylene binder (available under the trade name Tyrin QX 2243.25), 180 ml. toluene, .025 gram of Rhodamine B dissolved in 5 ml. methylene chloride, and  $2.85 \times 10^{-3}$  chemical equivalents of the zinc salt of the carboxylic acid ( $3.7 \times 10^{-6}$  equivalents per meter $^2$  of titanium dioxide), and  $2.85 \times 10^{-3}$  chemical equivalents of zinc oxide, as shown in Table 1.

Photoconductive copy sheets of each of these compositions are prepared by applying a uniform coating (about .7 mil thick dry) of the dispersion to a 1 mil thick film of polyethylene terephthalate (resistivity of  $10^{16}$  ohms/

square) having a thin vapor deposited aluminum coating (surface resistivity 5 ohms/square) on the underside and drying at room temperature. These steps are conducted under safelight conditions.

The sheets are then processed according to the electropowder process described in U.S. application Ser. No. 668,183. Process conditions are: 1500 volts, development voltage, 30 mil development gap, 15 mil doctor blade gap, temperature and humidity as shown in Table 1. The developer powder is a thermoplastic, electrically conductive, magnetically attractable powder ranging from 2-12 microns in diameter available under the trade name Type 842 Imaging Powder. The electrographic sheets are exposed to a tungsten iodide light for the optimum exposures for each sheet. The image densities (I.D.) of the test sheets are measured in the standard manner with a Macbeth Reflection Densitometer (Model RD-100) with the results shown in Table 1.

TABLE 1

| Example | Additives        | I.D. max.  |            |            |            |
|---------|------------------|------------|------------|------------|------------|
|         |                  | 70° F./50% | 80° F./62% | 80° F./71% | 81° F./81% |
| 1       | Zn acetate/ZnO   | 0.97       | 0.82       | 0.06       | 0          |
| 2       | Zn acetate       | 0.95       | 0.34       | 0          | 0          |
| 3       | Zn butyrate/ZnO  | 1.02       | 0.88       | 0.45       | 0.03       |
| 4       | Zn butyrate      | 0.95       | 0.06       | 0          | 0          |
| 5       | Zn hexanoate/ZnO | 0.98       | 0.78       | 0.10       | 0          |
| 6       | Zn hexanoate     | 0.91       | 0          | 0          | 0          |
| 7       | Zn octoate/ZnO   | 0.99       | 0.78       | 0.38       | .02        |
| 8       | Zn octoate       | 0.91       | 0          | 0          | 0          |
| 9       | Zn laurate/ZnO   | 0.92       | 0.56       | 0.01       | 0          |
| 10      | Zn laurate       | 0.64       | 0          | 0          | 0          |
| 11      | Zn stearate/ZnO  | 0.93       | 0.84       | 0.58       | .05        |
| 12      | Zn stearate      | 0.90       | 0.74       | 0.05       | 0          |
| 13      | Zn abietate/ZnO  | 1.05       | 0.99       | 0.97       | .96        |
| 14      | Zn abietate      | 1.04       | 1.00       | 0.91       | .06        |

## EXAMPLES 15-21

Dispersions are prepared as in the foregoing examples containing 38 grams titanium dioxide (characteristic relaxation time of 1.25 minutes), 12.6 grams of the binder of Example 1, 180 ml. toluene, .025 gram of Rhodamine B in 5 ml. methylene chloride,  $2.85 \times 10^{-3}$  equivalents (0.86 gram) abietic acid, and  $5.7 \times 10^{-3}$  equivalents of the metal oxide shown in Table 2.

Photoconductive sheets of the same construction as described in Examples 1-14 are prepared with these dispersions, and the resulting photoconductive sheets exposed and developed as in Examples 1-14 at the temperatures and humidities shown in Table 2. By comparison to the control (Example 21), the photoconductive sheets of this invention demonstrated an improvement in humidity resistance of the magnitude shown.

TABLE 2

| Example | Oxide            | I.D. max.    |              |
|---------|------------------|--------------|--------------|
|         |                  | (71° F./60%) | (80° F./85%) |
| 15      | BaO              | 0.94         | 0.88         |
| 16      | CaO              | 0.99         | 0.34         |
| 17      | MgO              | 0.96         | 0.30         |
| 18      | PhO              | 0.96         | 0.94         |
| 19      | HgO              | 1.00         | 0.99         |
| 20      | PbO <sub>2</sub> | 1.00         | 0.84         |
| 21      |                  | 0.94         | 0.00         |

## EXAMPLES 22-25

Electrographic sheets are prepared in accordance with the foregoing examples from 38 g. photoconductive titanium dioxide (trade name MS-540-5F), 12.6 g. of chlorinated polyethylene binder, 180 ml. toluene, 5 ml.

Rhodamine B dye (0.5% by volume in methylene chloride), carboxylic acid or salt thereof and zinc oxide in the amounts shown in Table 3. The sheets are processed according to the foregoing examples at the temperatures and humidities shown in Table 3, and the image density values obtained.

TABLE 3

| Example | Additives         | Equiva-                                                    | I. D. max. |            |
|---------|-------------------|------------------------------------------------------------|------------|------------|
|         |                   |                                                            | 72° F./51% | 80° F./80% |
| 22      | Abietic acid/ZnO  | $\{ 2.85 \times 10^{-3} \}$<br>$\{ 5.7 \times 10^{-3} \}$  | 0.99       | 0.83       |
| 23      | Abietic acid      | $2.85 \times 10^{-3}$                                      | 0.97       | 0.00       |
| 24      | Zinc rosinate ZnO | $\{ 2.85 \times 10^{-3} \}$<br>$\{ 2.85 \times 10^{-3} \}$ | 1.02       | 1.03       |
| 25      | Zinc rosinate     | $2.85 \times 10^{-3}$                                      | 1.02       | 0.92       |

From the data of the foregoing examples, it can be seen that the combination of the carboxylic acid or salt thereof and the metal oxide provides an image density greater than the corresponding image density obtained in the absence of the metal oxide at one or more humidity and temperature levels. The level at which the improvement is seen varies with the composition, as can be observed from the data. The environmental conditions employed in the tests are those which are encountered at various times of the year in nearly all countries. It is apparent that a drop in image density of the order shown constitutes a serious if not insurmountable barrier to general use of the electrographic process. The improvement in humidity resistance as reflected in image density of the photoconductive compositions of this invention appears to be observable at all levels of concentration of metal oxide and carboxylic acid or salt at one or more humidity levels. As the humidity is increased to the higher levels, the magnitude of the improvement increases.

Considerations other than humidity resistance may dictate limiting the quantity of carboxylic acid or salt and metal oxide. One factor in particular is the effect of such additives on light sensitivity. It has been observed that light sensitivity does decrease as the amounts of additives increases. Thus, for purposes of this invention, it is preferable that the quantities of additives be kept at or near the level where humidity resistance is satisfactory for the use at hand rather than increasing loading of the photoconductive composition beyond the satisfactory level to the detriment of other properties such as light sensitivity. To illustrate this point, the following examples are provided.

## EXAMPLES 26-33

Photoconductive compositions are prepared by the procedure of Examples 1-14 from the following ingredients plus the amount of zinc oxide and TiO<sub>2</sub><sup>1</sup> in Table 4:

|                                                        |    |      |
|--------------------------------------------------------|----|------|
| Polyethylene binder <sup>2</sup>                       | g  | 12.6 |
| Toluene                                                | ml | 180  |
| Rhodamine B (0.5% in CH <sub>2</sub> Cl <sub>2</sub> ) | ml | 5    |
| Abietic acid                                           | g  | 0.86 |

<sup>1</sup> Photoconductive titanium dioxide available under the trade name MS 540-5K.

<sup>2</sup> Trade name Tyrin (QX 2243.25).

Photoconductive sheets are prepared and tested as in Examples 1-14, the optimum exposure and image density at various conditions being shown in Table 4.

TABLE 4

| Example | Wt.<br>TiO <sub>2</sub> | Wt.<br>ZnO | Percent<br>ZnO | Exposure<br>(f.c.s.) | I.D. max.  |            |            |
|---------|-------------------------|------------|----------------|----------------------|------------|------------|------------|
|         |                         |            |                |                      | 80° F./66% | 80° F./72% | 80° F./85% |
| 26      | 38                      | 0          | 0              | 17.5                 | 0.48       | 0          | 0          |
| 27      | 38                      | 0.116      | .3             | 17.5                 | 0.89       | 0          | 0          |
| 28      | 37.6                    | 0.38       | 1              | 30                   | 0.97       | 0.01       | 0          |
| 29      | 36.1                    | 1.9        | 5              | 40                   | 0.99       | 0.98       | 0.92       |
| 30      | 34.2                    | 3.8        | 10             | 50                   | 1.01       | 1.00       | 0.92       |
| 31      | 30.4                    | 7.6        | 20             | 60                   | 0.99       | 0.98       | 0.94       |
| 32      | 19.0                    | 19.0       | 50             | 60                   | 1.06       | 1.09       | 1.05       |
| 33      | 9.5                     | 28.5       | 75             | 40                   | 1.13       | 1.16       | 1.14       |

7  
EXAMPLES 34-38

The following materials are introduced in the order listed into a 5 gal. container fitted with an air stirrer:

| Name:                                                 | Quantity            |
|-------------------------------------------------------|---------------------|
| Toluene                                               | g 6617              |
| Tyrin (Dow, QX 2743.25 trade name)                    | g 521               |
| Zinc rosinate (Union Camp, Univez 1028 trade name)    | g 38.7              |
| TiO <sub>2</sub> (National Lead, MS-540-5 trade name) | g 1562.7            |
| Rhodamine B                                           | g 1.03              |
| Methanol                                              | ml 200              |
| ZnO (USP-NJZ 12, trade name)                          | As shown in table 5 |

After premixing, the slurry is homogenized by 2 passes through the homogenizer (trade name Manton-Gaulin M-S15) at 3000 p.s.i. The dispersions thus prepared are allowed to cool to room temperature before coating.

The dispersions are then coated at a wet thickness of 3 mils on the polyester side of aluminum vapor coated 1 mil polyester film (dry coating thickness approximately 0.7 mil). Drying times of approximately 1/2 hour are required at ambient conditions.

The electrographic sheets are imaged and developed in the electropowder process at the humidities and temperatures shown in Table 5. The conditions for the electro-powder test machine are:

|                     |               |
|---------------------|---------------|
| Development voltage | +1500 volts.  |
| Development gap     | 0.035 in.     |
| Doctor blade gap    | 0.015 in.     |
| Development speed   | 16.5 in./sec. |

After development, the developer powder (same as in Examples 1-14) is fused to the electrographic sheet and the image density determined using a Macbeth RD-100 densitometer.

TABLE 5

| Example | Percent ZnO <sup>1</sup> | Exposure (f.c.s.) | I.D. max.  |            |            |            |            |
|---------|--------------------------|-------------------|------------|------------|------------|------------|------------|
|         |                          |                   | 80° F./54% | 80° F./61% | 80° F./68% | 80° F./75% | 80° F./80% |
| 34      | 0                        | 16                | 0.83       | 0.24       | 0          | 0          | 0          |
| 35      | 0.15                     | 16                | 0.97       | 0.83       | 0.34       | 0.02       | 0          |
| 36      | 0.30                     | 16                | 1.02       | 0.98       | 0.86       | 0.85       | 0.34       |
| 37      | 0.60                     | 20                | 1.04       | 1.04       | 1.03       | 1.03       | 1.02       |
| 38      | 3.0                      | 40                | 1.08       | 1.04       | 1.05       | 1.06       | 1.03       |

<sup>1</sup>By weight based on the combined weight of titanium dioxide and zinc oxide.

## EXAMPLES 39-43

Electrographic sheets are prepared and tested as in Examples 1-14 using the following ingredients:

|                                                                |                     |
|----------------------------------------------------------------|---------------------|
| TiO <sub>2</sub> (trade name 540-5K)                           | g 36.1              |
| ZnO (USP-12)                                                   | g 1.9               |
| Polyethylene binder (trade name Tyrin OX-2243.25)              | g 12.6              |
| Toluene                                                        | ml 180              |
| Rhodamine B (0.5% by vol. in CH <sub>2</sub> Cl <sub>2</sub> ) | ml 5                |
| Zn rosinate                                                    | As shown in Table 6 |

TABLE 6

| Example | Zn rosinate (equiv./in. <sup>2</sup> ) | TiO <sub>2</sub> surface) | Exposure (f.c.s.) | I.D. max.  |            |            |            |            |
|---------|----------------------------------------|---------------------------|-------------------|------------|------------|------------|------------|------------|
|         |                                        |                           |                   | 72° F./42% | 80° F./57% | 80° F./64% | 80° F./76% | 80° F./83% |
| 39      | 0                                      |                           | 20                | 0.94       | 0          | 0          | 0          | 0          |
| 40      | 0.92×10 <sup>-6</sup>                  |                           | 20                | 1.06       | 0.42       | 0.02       | 0          | 0          |
| 41      | 1.88×10 <sup>-6</sup>                  |                           | 20                | 1.07       | 1.01       | 0.91       | 0.01       | 0          |
| 42      | 3.7×10 <sup>-6</sup>                   |                           | 25                | 1.10       | 1.07       | 1.09       | 1.04       | 0.93       |
| 43      | 7.4×10 <sup>-6</sup>                   |                           | 40                | 1.14       | 1.16       | 1.16       | 1.09       | 1.06       |

In addition to improvements in humidity resistance, it has also been observed that electrographic elements bearing a surface coating of the formulations of this invention are capable of improving both reusability of the elements and imaging life, i.e., the ability to achieve multiple copies per exposure of the electrographic element.

What is claimed is:

1. A photoconductive composition comprising photoconductive titanium dioxide disposed in an insulating binder, said titanium dioxide being present to the extent of about 20 to about 80 volume percent of the combined volume of titanium dioxide and binder, a first additive of a carboxylic acid or metal salt thereof present to the extent of at least about  $1.85 \times 10^{-6}$  equivalents per square meter of titanium dioxide surface area, and a second additive of an inorganic metal oxide other than titanium dioxide present to the extent of at least about one-half of the equivalents thereof of said carboxylic acid or metal salt thereof and less than 20% by weight based on the combined weight of titanium dioxide and inorganic metal oxide.
2. The composition of claim 1 wherein said carboxylic acid or metal salt thereof is present to the extent of at least about  $3.7 \times 10^{-6}$  equivalents per square meter of titanium dioxide and said inorganic metal oxide other than titanium oxide is present to the extent of about one-half the chemical equivalents of said carboxylic acid or salt thereof.
3. The composition of claim 1 wherein said carboxylic acid or metal salt thereof is present in an amount sufficient to provide at least a monomolecular layer thereof on said titanium dioxide.
4. The composition of claim 1 wherein said carboxylic acid or metal salt thereof has from 2 to about 30 carbon atoms.
5. The composition of claim 1 wherein said first additive is a zinc salt of a carboxylic acid and said second additive is zinc oxide.
6. The composition of claim 1 wherein said first additive is a carboxylic acid or zinc salt thereof having from 6 to 20 carbon atoms, and said inorganic metal oxide is zinc oxide.
7. The composition of claim 1 wherein said inorganic

metal oxide is at least one member selected from the class consisting of barium oxide, calcium oxide, magnesium oxide, lead (II) oxide, lead (IV) oxide, mercuric oxide, and zinc oxide.

8. The composition of claim 1 wherein said first additive is an organic carboxylic acid or ammonium or metal salt thereof having 6 to 20 carbon atoms and said second additive is at least one inorganic metal oxide selected from the class consisting of barium oxide, calcium oxide, magnesium oxide, lead (II) oxide, lead (IV) oxide, mercuric oxide, and zinc oxide.

9. A photoconductive composition comprising an in-

sulating resin binder having distributed therein photoconductive titanium dioxide, said titanium dioxide being present to the extent of about 20 to about 80% by volume based on the combined volume of said titanium dioxide and insulating resin binder, a first additive of a carboxylic acid or metal salt thereof present to the extent of at least

about  $1.85 \times 10^{-6}$  equivalents per square meter of titanium dioxide surface area, and a second additive of an inorganic metal oxide other than titanium dioxide present to the extent of at least about one-half of the equivalents thereof of said carboxylic acid or metal salt thereof and less than 20% by weight based on the combined weight of titanium dioxide and inorganic metal oxide.

10. The composition of claim 9 wherein said carboxylic acid or metal salt thereof is present in an amount sufficient to provide at least a monomolecular layer thereof on said titanium dioxide.

11. The composition of claim 10 wherein said first additive is a zinc salt of a carboxylic acid and said second additive is zinc oxide.

12. The composition of claim 10 wherein said first additive is a carboxylic acid or zinc salt thereof having from 6 to 20 carbon atoms, and said inorganic metal oxide is zinc oxide.

13. An electrographic sheet having a surface layer comprising an insulating resin binder having distributed therein photoconductive titanium dioxide, said titanium dioxide being present to the extent of about 20 to about 80% by volume based on the combined volume of said titanium dioxide and insulating resin binder, a first additive of a carboxylic acid or metal salt thereof present to the extent of at least about  $1.85 \times 10^{-6}$  equivalents per square meter of titanium dioxide surface area, and a second additive of an inorganic metal oxide other than titanium dioxide, said surface layer being bonded to a dielectric layer present to the extent of at least about one-half of the equivalents thereof of said carboxylic acid or metal salt thereof and less than 20% by weight based on the combined weight of titanium dioxide and inorganic metal oxide.

14. The sheet of claim 13 wherein said inorganic metal oxide is at least one member selected from the class consisting of barium oxide, calcium oxide, magnesium oxide, lead (II) oxide, lead (IV) oxide, mercuric oxide, and zinc oxide.

15. An electrographic sheet having a surface layer comprising an insulating resin binder having distributed therein photoconductive titanium dioxide, said titanium dioxide being present to the extent of about 20 to about 80% by volume based on the combined volume of said titanium dioxide and insulating resin binder, a first additive of a carboxylic acid or metal salt thereof present to the extent of at least about  $1.85 \times 10^{-6}$  equivalents per square meter of titanium dioxide surface area, and a second additive of an inorganic metal oxide other than titanium dioxide present to the extent of at least about one-half of the equivalents thereof of said carboxylic acid or metal salt thereof and less than 20% by weight based on the combined weight of titanium dioxide and inorganic metal oxide, said surface layer being bonded to a dielectric layer and a conductive layer bonded to the underside of said dielectric layer.

16. A photoconductive composition comprising photoconductive titanium dioxide disposed in an insulating binder, said titanium dioxide being itself present to the

extent sufficient to provide a developable image in an electrographic process, a first additive of a carboxylic acid or metal salt thereof present to the extent of at least about  $1.85 \times 10^{-6}$  equivalents per square meter of titanium dioxide surface areas, and a second additive of an inorganic metal oxide other than titanium dioxide present to the extent of at least about one-half of the equivalents thereof of said carboxylic acid or metal salt thereof and less than 20% by weight based on the combined weight of titanium dioxide and inorganic metal oxide.

17. An electrographic sheet having a surface layer comprising photoconductive titanium dioxide disposed in an insulating resin binder, said titanium dioxide being itself present to the extent sufficient to provide a developable image in an electrographic process, said titanium dioxide being present to the extent of about 20 to about 80% by volume based on the combined volume of said titanium dioxide and insulating resin binder, a first additive of a carboxylic acid or metal salt thereof present to the extent of at least about  $1.85 \times 10^{-6}$  equivalents per square meter of titanium dioxide surface area, and a second additive of an inorganic metal oxide other than titanium dioxide present to the extent of at least about one-half of the equivalents thereof of said carboxylic acid or metal salt thereof and less than 20% by weight based on the combined weight of titanium dioxide and inorganic metal oxide, said surface layer being bonded to a dielectric layer.

#### References Cited

##### UNITED STATES PATENTS

|           |         |                       |           |
|-----------|---------|-----------------------|-----------|
| 3,198,632 | 8/1965  | Kimble et al. -----   | 96—1      |
| 3,079,253 | 2/1963  | Greig -----           | 96—1      |
| 3,220,830 | 11/1965 | Kashiwabana -----     | 96—1.8    |
| 3,245,784 | 4/1966  | Stricklin -----       | 96—1.8    |
| 3,248,217 | 4/1966  | Shulman -----         | 96—1.8    |
| 2,901,348 | 8/1959  | Dessauer et al. ----- | 96—1.5    |
| 3,241,458 | 3/1966  | Borhardt et al. ----- | 96—1.8    |
| 3,174,856 | 3/1965  | Horne et al. -----    | 96—1.8    |
| 3,234,017 | 2/1966  | Heyl et al. -----     | 252—501 X |
| 3,378,371 | 4/1968  | Jarvis -----          | 96—1.8    |
| 3,418,147 | 12/1968 | Fields -----          | 106—300 X |
| 3,492,264 | 1/1970  | Hahn -----            | 106—309 X |
| 3,561,968 | 2/1971  | Dantro -----          | 252—501 X |
| 3,632,527 | 1/1972  | Alpert et al. -----   | 252—501   |
| 3,607,262 | 9/1971  | Veda -----            | 96—1.8    |
| 3,569,803 | 3/1971  | Sato et al. -----     | 96—1.8 X  |
| 3,653,895 | 4/1972  | Brandon -----         | 96—1.8    |

##### OTHER REFERENCES

50 Klein, Otto C.: Effect of Moisture and Type of Binder on Electrophotographic Behavior, TAPPI, vol. 47, No. 9, September 1964, pp. 145—148.

55 CHARLES E. VAN HORN, Primary Examiner

U.S. Cl. X.R.

96—1.5; 252—501

UNITED STATES PATENT OFFICE  
CERTIFICATE OF CORRECTION

Patent No. 3,736,134 Dated May 29, 1973

Inventor(s) Donald W. Gosselink and Einar D. Horne

It is certified that error appears in the above-identified patent  
and that said Letters Patent are hereby corrected as shown below:

Col. 1, line 51, "or" should read -- of --.

Col. 2, lines 28,29, in the table,

|              |            |             |              |            |
|--------------|------------|-------------|--------------|------------|
| 80°/80% .... | 0.76 O.D.U | should read | 80°/61% .... | 0.76 O.D.U |
| 80°/61% .... | 0          |             | 80°/80% .... | 0          |

Signed and sealed this 21st day of May 1974.

(SEAL)

Attest:

EDWARD M. FLETCHER, JR.  
Attesting Officer

C. MARSHALL DANN  
Commissioner of Patents